

## UNITED STATES PATENT OFFICE

2,220,891

AMMONIUM NITRATE EXPLOSIVE  
COMPOSITION

Melvin Alonzo Cook, Clyde Oliver Davis, and  
Walter Eastby Lawson, Woodbury, N. J., as-  
signors to E. I. du Pont de Nemours & Company,  
Wilmington, Del., a corporation of Delaware

No Drawing. Application August 9, 1939,  
Serial No. 289,187

8 Claims. (Cl. 52—14)

This invention relates to new and improved ammonium nitrate explosive compositions, and more particularly to such ones as can be packed to high densities and which possess superior sensitiveness properties at such high densities.

It is well known that ammonium nitrate constitutes an effective blasting agent when blended with combustible materials in amounts sufficient to give oxygen-balanced compositions and with a satisfactory sensitizing agent. While nitroglycerin has been the most commonly-used sensitizer, very efficient blasting explosives are in regular production comprising ammonium nitrate blended with solid, non-explosive sensitizing ingredients capable of utilizing the excess oxygen of the ammonium nitrate for their own complete combustion.

In the case of ammonium nitrate high explosives sensitized by means of non-explosive solid sensitizers, very careful control and handling are necessary in order that the product shall maintain its explosive properties unimpaired during storage. The affinity of ammonium nitrate for water makes this particularly important, since ammonium nitrate has a tendency to become hard and insensitive in the presence of even small amounts of water.

The object of the present invention is an explosive composition of high ammonium nitrate content, possessing outstanding properties. A further object is such an explosive characterized by high density and of a high order of sensitiveness for an ammonium nitrate explosive of such high density. Additional objects will be disclosed as the invention is described more at length hereinafter.

The foregoing objects are accomplished, and the disadvantages of the prior art overcome, by the formulation of explosive compositions containing ammonium nitrate as the predominant ingredient, a sensitizer for the ammonium nitrate, an inorganic nitrate, and combined ammonia. By combined ammonia we mean combined molecular ammonia.

We find it desirable to employ in the compositions of our invention an inorganic nitrate which is capable of reacting with gaseous ammonia, for example to form a metal ammine, an ammoniate, or other ammonia addition compound. In other words, this essential inorganic nitrate is one other than the nitrates of the alkali metals, since the latter failed to form said addition compounds with ammonia. By the term "ammine" we are not referring to the organic amines, but to the well-recognized inorganic compounds con-

taining combined molecular ammonia, frequently referred to as the ammoniates, or as the metal amines, or synonymously as an inorganic compound containing ammonia of crystallization. Discussion of compounds of this type, for example, is found in Friend's "Textbook of Inorganic Chemistry." Volume 10 of the same is devoted entirely to the metal amines. The compounds are also referred to in the book by Franklin, "Nitrogen System of Compounds", page 38. The latter term has been employed by Edward C. Franklin on page 38 of his book entitled "The Nitrogen System of Compounds".

Ammonium nitrate should be present as the preponderant ingrédient, that is in an amount greater than 50%. Preferably, however, our compositions will contain more than 75% ammonium nitrate. Various sensitizers for the ammonium nitrate may be used which are capable of oxidation by, and of utilizing at least a portion of, the excess oxygen of the ammonium nitrate. The nitroaromatic hydrocarbons and compounds comprise very desirable sensitizers, particularly the nitrotoluenes. Other organic sensitizers than the nitrotoluenes are available and applicable, however, for example the various nitronaphthalenes, diphenylamine, diphenyl and the like. It will be understood also that inorganic sensitizers may be used, such as aluminum, sulfur, calcium silicide, ferrosilicon, and the like.

The compositions according to our invention, as has been stated, will contain more than 50% ammonium nitrate and preferably more than 75%. The organic sensitizer will desirably be present in an amount between 0.5 and 20.0%, dinitrotoluene being our preferred material. The reaction product of the inorganic metal nitrate and ammonia should be present in an amount between 0.1 and 10.0%.

Various methods are available for preparing the explosive compositions according to our invention, especially those described in our co-pending application, Serial No. 289,188, dated Aug. 9, 1939. According to our preferred method, calcium cyanamide is heated to a temperature around 80° C. with a blend of ammonium nitrate and dinitrotoluene, whereby gaseous ammonia is given off as a reaction product and calcium nitrate is formed. The ammonia reacts with the calcium nitrate, presumably to form a calcium nitrate ammine. Both the initial product, calcium cyanamide and calcium nitrate, are fusion point depressants for the ammonium nitrate. The organic sensitizer should be one having a melting point such that the material is at least

partly fused at the temperature of mixing of the explosion; hence it should desirably have a fusion point below 100° C.

We find the advantages of the presence of the reaction product of ammonia with calcium nitrate or other metal nitrate other than those of the alkali metals to be especially important in the case of high density blends of ammonium nitrate and sensitizer. It is with compositions having a density above 1.15, for example between 1.15 and 1.7, that we find our invention most effective. Compositions of such high density are very desirable in quarry blasting where it is important to secure the maximum blasting effect. Certain ammonium nitrate explosives are now in use which contain only non-explosive sensitizers. These are relatively insensitive explosives. Some are so much so that they are incapable of detonation by a commercial blasting cap, though they can be readily detonated and caused to propagate with undiminished high velocity, when initiated by a suitable booster charge of trinitrotoluene or other high explosive. With such explosives, densities greater than 1.15 are frequently impractical, since there is too great a chance of failure to detonate. Utilizing the compositions of the present invention, however, densities much higher than 1.15 are utilizable. Preferably the explosive will be enclosed in a completely water-tight and air-tight container such as a metal can. Under such conditions the composition is protected completely against moisture.

As examples of explosive compositions according to our invention, the following will serve:

35

#### Example I

An explosive composition was prepared, which comprised 84% ammonium nitrate, 12% dinitrotoluene, and 4% calcium nitrate. The maximum density at which propagation of the explosive could be continuously effected was found to be 1.25. The velocity of detonation at this density was determined to be 1750 meters per second. This example contained no free ammonia for combination with the calcium nitrate, and the relative insensitiveness and low velocity are apparent.

#### Example II

The explosive composition of this example comprised 83% ammonium nitrate, 12% dinitrotoluene, and 5% of a compound of calcium nitrate and ammonia, which may be designated



The increased sensitiveness, due to the presence of the reaction product of ammonia and the calcium nitrate, can be seen from the maximum propagating density of over 1.35, in comparison with 1.25 for the composition of Example I. Moreover the velocity of this composition at a density of 1.30 was 3830 meters per second.

#### Example III

The explosive composition comprised 81.5% ammonium nitrate, 12.0% dinitrotoluene, and 6.5% of the reaction product of barium nitrate and ammonia. The maximum density at which continuous propagation took place was 1.30, in comparison with 1.22 for a similar composition containing simply barium nitrate instead of its addition product with ammonia. The velocity of the composition of this example was 3500 meters per second at a density of 1.30, whereas for the similar explosive containing only barium nitrate the velocity was 2250 at a density of 1.22.

#### Example IV

The composition comprised 81.5% ammonium nitrate, 12.0% dinitrotoluene, and 6.5% of the reaction product of strontium nitrate with ammonia. The improvement effected by the presence of this reaction product is shown by the fact that the composition of this example has a maximum propagating density of 1.27 against 1.21 for a similar composition containing only strontium nitrate. Likewise improved velocity was shown, 3325 meters per second at a density of 1.25 against 1900 meters at 1.20.

#### Example V

A composition was prepared comprising approximately 81.5% ammonium nitrate, 12.0% dinitrotoluene, and 6.5% of a reaction product of hydrated cupric nitrate and ammonia. The explosive at a density of 1.30, in metal containers of 2" diameter, gave consistently high velocity detonations, when properly primed. The efficacy of the ammonia addition product was shown from the fact that a similar composition containing cupric nitrate, not ammoniated, failed to detonate at a density of 1.20.

Various inorganic nitrates and other salts are available which are effective in increasing the sensitiveness of the high ammonium nitrate compositions of our invention. Such salts include calcium nitrate, barium nitrate, strontium nitrate, zinc nitrate, lead nitrate, cobalt nitrate, copper nitrate, cobalt perchlorate, and the like. While we have excluded the nitrates of the alkali metals from our invention with respect to compounds with ammonia, it should be understood that sodium nitrate or other alkali nitrate may be present in the role of oxidizing agent or other capacity. Likewise many other ingredients may be included.

It has been stated previously that we may apply our invention effectively in the case of cap-insensitive explosives which are capable of detonation by a booster charge, whereby these blasting agents are made more certainly detonable. It may likewise be utilized to sensitize cap-insensitive compositions and make them sensitive to commercial blasting caps. Furthermore, it is applicable in the case of certain explosives of high ammonium nitrate content which thereby become practical for use in smaller diameters than would otherwise be possible.

We have described our invention at length in the foregoing, but it will be understood that many variations may be introduced without departure from the scope of the invention. We wish to be limited, therefore, only by the following patent claims:

We claim:

1. An ammonium nitrate explosive composition having a density greater than 1.15, said composition comprising more than 50% ammonium nitrate, a sensitizer therefor, an inorganic nitrate other than those of the alkali metals, and molecular ammonia combined therewith.

2. An ammonium nitrate explosive composition having a density greater than 1.15, said composition comprising more than 50% ammonium nitrate, an organic sensitizer for the ammonium nitrate, and the reaction product of ammonia with an inorganic metal nitrate other than those of the alkali metals.

3. An ammonium nitrate explosive composition having a density greater than 1.15, said composition comprising more than 50% ammonium nitrate, an organic sensitizer therefor, and

an ammine of an inorganic nitrate other than those of the alkali metals.

4. An ammonium nitrate explosive characterized by high density, said composition comprising more than 50% ammonium nitrate, an organic sensitizer for said ammonium nitrate, and the reaction product of ammonia with calcium nitrate.

5. An ammonium nitrate explosive composition having a density greater than 1.15, said composition comprising more than 75% ammonium nitrate, between 0.5 and 20.0% of an organic sensitizer therefor, and between 0.1 and 10.0% of the reaction product of ammonia with a metal nitrate other than those of the alkali metals.

6. An ammonium nitrate explosive composition characterized by high density and of a degree of sensitiveness such that it is incapable of detonation by a commercial blasting cap but can

be detonated by means of a suitable booster charge, said composition comprising more than 75% ammonium nitrate, between 0.5 and 20.0% of an aromatic nitrocompound, and between 0.1 and 10.0% of the reaction product of ammonia with calcium nitrate.

7. The explosive composition of claim 6, in which the aromatic nitrocompound is dinitrotoluene.

8. An ammonium nitrate explosive comprising more than 50% ammonium nitrate and an inorganic nitrate other than those of the alkali metals containing ammonia of crystallization combined with said nitrate, said compound being intimately dispersed within the body of the ammonium nitrate as a sensitizer for the latter.

MELVIN ALONZO COOK.

CLYDE OLIVER DAVIS.

WALTER EASTBY LAWSON.